

# UNITED STATES PATENT OFFICE.

JAMES ROWE, OF SAN FRANCISCO, CALIFORNIA.

## COMPOSITION FOR PROTECTING PILES.

SPECIFICATION forming part of Letters Patent No. 440,832, dated November 18, 1890.

Application filed September 19, 1890. Serial No. 365,551. (No specimens.)

*To all whom it may concern:*

Be it known that I, JAMES ROWE, a citizen of the United States, residing in the city and county of San Francisco, State of California, 5 have invented an Improvement in Pile-Protecting Compositions; and I hereby declare the following to be a full, clear, and exact description of the same.

My invention relates to that class of pile- 10 protectors which consists of suitable compositions of matter applied to the exterior of the pile and forming a covering therefor which is intended to resist not only the action of the water, but especially the ravages of marine insects, particularly the teredo.

My invention consists in an inner covering 15 and an outer coating. The inner covering consists of the following ingredients, combined in substantially the proportions stated, 20 to wit: tar, five gallons; asphalt, one hundred and fifty pounds; paraffine, fifty pounds; cement, twenty-five pounds; phosphorus, one pound; hair, five pounds. The manner of mixing these is as follows: The tar is put in 25 a kettle and raised to the boiling-point. The asphalt is then put into the kettle and well stirred in with the tar, the boiling being continued until the mass is thoroughly reduced to a liquid form—say for about an hour. The 30 paraffine is next added, and the mass is stirred while boiling over a slow fire for, say, three hours, or thereabout. The proportion of paraffine need not be absolutely that above given. So much is put in as will give the proper 35 hardness to the mass when set. The cement is then added to thicken the mass to suit. The fire is then drawn, and the hair is immediately put in and stirred well. Horse-hair is preferable, though cow-hair may be used. 40 Then the phosphorus is added and well stirred. The pile is now placed over the kettle, being mounted upon suitable wheeled frames or trucks, and the material in the kettle is mopped up around the pile until it covers it 45 to proper thickness—say from one-quarter to one-half inch, or thereabout. Then the pile is rolled over to one side on skids and left to dry, say, for three days. The covering in this time becomes perfectly hard and sticks firmly

and closely to the wood. The outer coating 50 consists of fire-clay, sand, and cement mixed in such proportions as to make the mass of the consistency of molasses, approximately. This is then applied to the covering of the pile with a brush or broom, and the pile is left for 55 about a week, so that the coating will set.

In this protector the hair plays an important part, its function being not only to serve as a bond, but also to act as a barrier or resistant to the worm. Its keenness or fineness 60 of edge causes it to act as a cutter, and it splits the boring organ of the worm, deterring it from further advancing. The phosphorus serves as a poison and kills the worm. This covering is very hard of itself and will resist 65 the sun's rays. The paraffine gives it this quality, so much being put in as will give the mass the essential consistency and yet not allow it to soften under any heat to which the pile while in use may be exposed. The cement 70 serves to further harden the mass. The tar is the liquefying or melting element, and linseed-oil may be substituted for it, though tar is preferable, being cheaper. The asphalt forms the body of the mass. The outer coating is essential to perfect durability. It hardens the whole; but its chief function is to protect the inner covering, holding it to place and shielding it from the sun's rays, thereby 75 not only protecting the inner mass as a whole, 80 but fully shielding the phosphorus.

I am aware that in pile-protectors many of the foregoing ingredients—such as tar, asphalt, cement, and paraffine—have been used separately or in combination with other substances; but I am not aware that they have been combined as I have herein set forth, nor with phosphorus and hair. Therefore, 85

What I claim as new, and desire to secure 90 by Letters Patent, is—

1. A pile-protecting composition consisting of tar, asphalt, paraffine, cement, phosphorus, and hair, substantially as herein described.

2. A pile-protecting composition consisting of an inner covering of a composition of tar, asphalt, paraffine, cement, phosphorus, and hair, and an outer coating of a plastic material or composition which will harden or set 95

after being applied, substantially as herein described.

3. A pile-protecting composition consisting of an inner covering of a composition of tar, asphalt, paraffine, cement, phosphorus, and hair, and an outer coating of a composition of fire-clay, sand, and cement, substantially as herein described.

In witness whereof I have hereunto set my hand.

JAMES ROWE.

Witnesses:

S. H. NOURSE,  
H. C. LEE.